

# UNITED STATES PATENT OFFICE.

JAMES F. SALLows, OF LANSING, MICHIGAN, ASSIGNOR TO ALFRED O. BLAICH, OF CHICAGO, ILLINOIS.

## CASE-HARDENING MIXTURE.

1,079,954.

Specification of Letters Patent.

Patented Dec. 2, 1913.

No Drawing.

Application filed December 26, 1912. Serial No. 738,703.

*To all whom it may concern:*

Be it known that I, JAMES F. SALLows, a citizen of the United States, residing at Lansing, in the county of Ingham and State 5 of Michigan, have invented certain new and useful Improvements in Case-Hardening Mixtures, of which the following is a specification.

This invention relates to material for use 10 in cementing or case-hardening.

Most mixtures employed for the purpose of cementation or case-hardening by dry packing comprise as the essential element from which the carbon is to be derived, some 15 comparatively costly substance, such as bone-dust or powdered charred leather charcoal. I have discovered, however, that the spent tan bark commonly known as tan waste, which is a by-product of ordinary tanning 20 processes and which has hitherto been considered of no value, is rendered exceptionally effective for the purpose of cementation when used in conjunction with the energizing substances commonly employed, which 25 are salts of alkaline bases such as sodium carbonate, barium carbonate and ammonium carbonates, slaked lime being preferably added with some of these salts and permissible with any of them.

30 A very effective mixture for the purpose consists of from 65 to 70 per cent. of the tan waste above mentioned, preferably powdered and intimately mixed with from 12 to 15 per cent. of barium carbonate, about 5 per 35 cent. of soda ash, from 8 to 10 per cent. of slaked lime and about  $2\frac{1}{2}$  per cent. of ammonium carbonate. If it is preferred to avoid the unpleasantness of the use of sodium carbonate, I find that about 10 per 40 cent. of common salt may be substituted for this element of the combination. When properly mixed and used in the ordinary manner, that is, by embedding the article to be case-hardened in the mixture and heating 45 to incandescence, the resulting surface will contain as high as 1.35 per cent. carbon as compared with about .80 per cent., which is about the limit of carbonization obtainable with ordinary mixtures now in use. And,

on account of the absence of other uses for 50 the tan waste which is the principal ingredient of the mixture, this material is both cheap and abundant.

When any of the sodium salts mentioned 55 is employed, the use therewith of the slaked lime has the effect of retaining the chemical elements which would otherwise pass off in vapor so that they may produce their desired effect in combination with the carbonaceous matter.

60 The tan waste can be used either charred or not charred. The advantage of charring is reduction of volume so that there is less shrinkage of the mixture in use. There is always more or less fine dust with the tan 65 waste and this is especially true when it is charred, and on this account I prefer to spray it with oil,—hydro-carbon oil being preferred,—before mixing it with the elements. The amount of oil used should be 70 only such as to lay the dust without making the mixture wet.

I claim:

1. A case-hardening mixture consisting principally of tan bark combined in physical mixture with energizing material comprising salts of an alkaline base for rendering the carbonaceous matter of the tan bark active when the mixture is heated.

2. A case-hardening mixture consisting 80 principally of carbonaceous material in the form of spent tan bark combined in physical mixture with energizing material comprising a sodium salt and slaked lime to render the carbonaceous matter active when the 85 mixture is heated.

3. A case-hardening mixture consisting principally of carbonaceous material in the form of spent tan bark mixed with energizing substance, including barium carbonate, 90 a sodium salt, slaked lime and ammonium carbonate.

4. A case-hardening mixture consisting of from 65 to 70 per cent. spent tan bark, 12 to 15 per cent. barium carbonate, 5 to 10 per 95 cent. of a sodium salt, 8 to 10 per cent. slaked lime, and about  $2\frac{1}{2}$  per cent. ammonium carbonate.

5. A case-hardening mixture consisting of  
from 65 to 70 per cent. spent tan bark, 12 to  
15 per cent. barium carbonate, approximately  
10 per cent. sodium chlorid, 8 to 10 per cent.  
slaked lime, and about 2½ per cent. ammo-  
nium carbonate.

In testimony whereof I have hereunto set

my hand at Lansing, Michigan, this 14th  
day of December, 1912.

JAMES F. SALLOWS.

Witnesses:

CHAS. W. FOSTER,  
NETTIE KULL.